

June 26, 1945.

H. L. BODE

2,378,972

PROCESS OF PRODUCING GREASE PACKAGES

Filed May 4, 1942



INVENTOR:

Harry L. Bode,  
by Carl H. Gravely,

HIS ATTORNEY

## UNITED STATES PATENT OFFICE

2,378,972

PROCESS OF PRODUCING GREASE  
PACKAGESHarry L. Bode, Webster Groves, Mo., assignor to  
Gaylord Container Corporation, St. Louis, Mo.,  
a corporation of Maryland

Application May 4, 1942, Serial No. 441,602

6 Claims. (Cl. 226—19)

This invention relates to the packaging of grease, especially grease that is used for lubricating purposes. Grease is usually shipped in metal or wood containers which are relatively expensive. It has a tendency to stick to such containers so that a portion thereof must be left in the container or scraped out at the risk of getting into the grease extraneous matter that impairs its value as a lubricant. Paperboard containers would be much cheaper but are open to the objection that paper absorbs grease and thereby becomes unsightly and dirty. This statement applies not only to untreated paper and paperboard but also to paper and paperboard coated with any of the usual paraffin coating compositions used for rendering the paper impermeable to ordinary liquids. The principal object of the present invention is to devise a satisfactory paperboard container for grease and to devise a method of packaging grease therein. The invention consists principally in coating the inside of a paperboard container with a paraffin wax-in-water emulsion containing graphite in suspension and then pouring melted grease into the container. It also consists in the container coated with said composition and dried and also in the package consisting of the container with the grease melted therein. It also consists in specific details hereinafter described and claimed.

In the accompanying drawing, wherein like reference numerals refer to like parts wherever they occur,

Fig. 1 is a view partly in section and partly in elevation of a paperboard container prior to having its inner surface coated with a wax-in-water emulsion containing graphite.

Fig. 2 is a similar view of the container with its inner surface covered with a waxy coat containing graphite remaining after the water is eliminated and ready to receive the grease.

Fig. 3 is a similar view of a package consisting of the container with grease therein.

Fig. 4 is an enlarged fragmentary sectional view of the container wall with the wax-in-water coating freshly applied thereto.

Fig. 5 is a similar fragmentary view showing the coating after absorption and evaporation of the water content of the coating, that is, in a condition ready to receive the grease; and

Fig. 6 is a similar fragmentary view of the package showing the film of graphite intervening between the paperboard and the grease.

I start with a container 1 made of "paperboard," which term is used herein to include fiberboard, chipboard and similar material and

of any suitable shape. The inner surface of this container 1 is coated, as shown at 2a in Fig. 4 with a liquid composition consisting of a wax-in-water emulsion having finely divided graphite suspended therein. The greater portion of the water of the emulsion is absorbed by the cardboard leaving behind a film of wax and graphite as shown at 2b in Figs. 2 and 5. Then the container is permitted to dry. Melted grease 3 is then poured into the container with the result that the wax of the coating is melted and a portion thereof is absorbed into the wall of the container and the rest is absorbed by the melted grease. The graphite then remains behind as a barrier coat or film 2c between the grease and the wall of the container and functions to prevent the grease from being absorbed by the wall of the container and also functions to prevent or minimize the sticking of the grease to the wall of the container. Thus the initial wax-in-water emulsion serves as a temporary or fugitive vehicle or medium by which graphite can be applied as a thin continuous film between the grease and the wall of the container. The water component of the emulsion is evaporated and disappears. The wax component impregnates and waterproofs the paperboard without discoloring or impairing the outer surface thereof; and as the paraffin wax is similar in character to the grease, the qualities of the grease are not appreciably affected by the intrusion of wax into it. The graphite, which remains as a barrier film adheres more strongly to the paperboard than to the grease so that very little, if any, graphite gets into the grease; and as graphite is itself a superior lubricant, the value of the grease is not appreciably affected by a small content of graphite.

A wax-in-water emulsion that has given very satisfactory results in my composition, and which is hereinafter referred to as emulsion No. 1, consists of about 500 parts by weight of fully refined paraffin having a melting point of 135° F., about 70 parts by weight of triethanolamine, about 140 parts by weight of stearic acid and about 1060 parts by weight of water. The triethanolamine is an emulsifying agent that effectively disperses the wax in the water and the stearic acid combines with the emulsifying agent to form a soap that aids in emulsification. In preparing the emulsion, the paraffin and the stearic acid were melted and heated in a water bath to a temperature of 170° F. The triethanolamine was added to the emulsion water and the solution boiled and the paraffin and stearic acid solution were

then added with constant stirring until the liquid became cool. This produced an emulsion containing about sixty percent of water.

The following emulsion, hereinafter referred to as emulsion No. 2, has also been found to be very satisfactory, namely, about 500 parts by weight paraffin having a melting point of 135° F., about 35 parts by weight sodium silicate, about 140 parts by weight of stearic acid and about 2160 parts by weight of water, the sodium silicate being used as an emulsifying agent.

In preparing emulsion No. 2, the paraffin and stearic acid were melted and heated in a water bath to 170° F. The sodium silicate was dissolved in the emulsion water and this solution was heated to boiling. The hot paraffin-stearic acid mixture was slowly added to the boiling sodium silicate solution and constantly stirred until the mixture cooled. This produced an emulsion containing about 76% water.

When a harder final coating film is desired, carnauba wax may be used in combination with the paraffin. A suitable emulsion of this type, hereinafter designated emulsion No. 3, may be made with about 400 parts by weight of paraffin having a melting point of 135° F., about 100 parts by weight of carnauba wax, refined yellow, about 90 parts by weight of oleic acid, about 90 parts by weight of triethanolamine, about 10 parts by weight of borax and about 1600 parts by weight of water. The borax accelerates the action of the emulsifying agent and makes for better spreading qualities. This emulsion No. 3, contains about 70 percent of water.

In preparing emulsion No. 3, the paraffin and carnauba wax were heated together in a water bath and the temperature maintained at 205° F. While this 205° F. temperature was maintained, the oleic acid and triethanolamine were added to the hot wax mixture. The borax was dissolved in the emulsion water and this solution was brought to boiling, when it was added to the hot wax mixture, with constant stirring.

Various grades of finely divided graphite have been found satisfactory in connection with emulsions of the kind above specified. Thus, about 47 parts by weight of powdered amorphous graphite, No. 325 mesh size, graphitic carbon content 84 to 86 percent, may be used with about 95 parts by weight of emulsion No. 1, and the whole stirred to form a smooth, homogeneous mixture. Additional water, say ordinarily about 8 parts by weight of water, may be added in conformity with common practice to better adapt the composition to the particular method used in applying it to the container. Likewise, 17 parts by weight of flake graphite, 80 percent graphitic carbon, ground to retain about 30 percent on a No. 100 mesh sieve and averaging around 50 percent passing a No. 200 mesh sieve, and 17 parts by weight of powdered amorphous graphite, No. 325 mesh, graphitic carbon content 84 percent to 86 percent, may be used with 95 parts by weight of emulsion No. 1, with water added, if desired, to suit the method of application to the container, say about 4 parts by weight of water. Approximately the same amounts of graphite may be used with emulsions Nos. 2 and 3.

It is to be understood that the proportions of the emulsion ingredients hereinbefore specified are typical and subject to variation provided the graphite-containing composition has a consistency suitable for applying it to the paperboard by ordinary methods.

A graphite-containing wax-in-water emulsion

conforming substantially to the typical formulas hereinbefore set out may be applied to a paperboard container at the rate of from 300 to 500 square feet per gallon whereupon the water is quickly absorbed by the paperboard and evaporated, leaving a waxy coat. This coat contains enough graphite to form a continuous film when the wax is melted and passes by absorption into the grease and the wall of the container. The wax is beneficial to the paperboard and neither the wax nor the other ingredients are harmful to the grease. After the water and the wax are absorbed, the graphite remains as an effective barrier that keeps the grease from penetrating into the paperboard.

What I claim is:

1. The process of packaging grease and the like which comprises coating the inner surface of a paperboard container with a wax-in-water emulsion containing graphite in suspension, permitting said container to become substantially dry and then pouring the grease in melted condition into said container the temperature of said grease being high enough to melt said wax thereby causing it to penetrate said paperboard and said grease, leaving a film of graphite between the paperboard and the grease.

2. The process of packaging grease and the like which comprises coating the inner surface of a paperboard container with an emulsified composition consisting mainly of about 500 parts by weight of paraffin and 1060 parts by weight of water and containing about 930 parts of graphite, permitting said container to become substantially dry and then pouring the grease in melted condition into said container the temperature of said grease being high enough to melt said wax thereby causing it to penetrate said paperboard and said grease, leaving a film of graphite between the paperboard and the grease.

3. The process of packaging grease and the like which comprises coating the inner surface of a paperboard container with an emulsified composition consisting mainly of approximately 500 parts by weight of paraffin and 1060 parts by weight of water, an emulsifying agent and from 560 to 930 parts by weight of graphite, permitting said container to become substantially dry and then pouring the grease in melted condition into said container the temperature of said grease being high enough to melt said wax thereby causing it to penetrate said paperboard and said grease, leaving a film of graphite between the paperboard and the grease.

4. The process of packaging grease and the like which comprises coating the inner surface of a paperboard container with an emulsified composition consisting mainly of about 500 parts by weight of paraffin, and about 1060 parts by weight of water and an emulsifying agent consisting of about 70 parts by weight of triethanolamine and about 140 parts by weight of stearic acid and from about 560 to 930 parts by weight of graphite, permitting said container to become substantially dry and then pouring the grease in melted condition into said container the temperature of said grease being high enough to melt said wax thereby causing it to penetrate said paperboard and said grease, leaving a film of graphite between the paperboard and the grease.

5. The process of packaging grease and the like which comprises coating the inner surface of a paperboard container with an emulsified composition consisting of about 2160 parts by

weight of water, about 140 parts by weight of stearic acid, about 35 parts by weight of sodium silicate and from about 560 to about 930 parts by weight of graphite, permitting said container to become substantially dry and then pouring the grease in melted condition into said container the temperature of said grease being high enough to melt said wax thereby causing it to penetrate said paperboard and said grease, leaving a film of graphite between the paperboard and the grease.

6. The process of packaging grease and the like which comprises coating the inner surface of a paperboard container with an emulsified composition consisting mainly of about 400 parts

by weight of paraffin, about 100 parts by weight of carnauba wax, about 90 parts by weight of oleic acid, about 90 parts by weight of triethanolamine, about 10 parts by weight of borax and about 1600 parts by weight of water and 620 to 860 parts by weight of graphite, permitting said container to become substantially dry and then pouring the grease in melted condition into said container the temperature of said grease being high enough to melt said wax thereby causing it to penetrate said paperboard and said grease, leaving a film of graphite between the paperboard and the grease.

HARRY L. BODE.